

1

3,000,807

## BLENDED TRANSFORMER OIL

Jones L. Wasson, Union, and James E. Kehoe, Clark, N.J.,  
assignors to Esso Research and Engineering Company,  
a corporation of Delaware  
No Drawing. Filed Dec. 4, 1958, Ser. No. 778,085  
6 Claims. (Cl. 208—14)

This invention is concerned with an improved transformer oil comprising a blend of two select base stocks. More particularly it is concerned with a transformer oil consisting essentially of a blend of an acid treated distillate and a hydrofined distillate which blend surprisingly has a higher uninhibited Doble Oxidation Test life than either of its components.

A major factor in the market acceptance of a transformer oil is good oxidation resistance without the use of added inhibitors. Users of transformer oils have traditionally used uninhibited oils and are suspicious of oils containing inhibitors unless it is known that the base oil itself has good oxidation resistance. This feeling is firmly entrenched. It is due partly to a belief that an inhibitor can be destroyed in the oil or volatilized by severe heat or extreme overloads, and partly to a fear that the oils made by inhibiting the poor base stock give insufficient warning of a coming breakdown. Thus, while it is not clear how the oxidation resistance of an uninhibited transformer oil relates to its performance in use with an inhibitor, it is clear that in order to have a saleable and marketable product, the base oils used in the transformer oil must show excellent uninhibited oxidation resistance. This oxidation resistance is customarily tested by the conventional Doble Oxidation Test for electrical insulating oils developed by the Doble Engineering Company of Belmont, Massachusetts.

In the Doble oxidation test an oil heated to 95° C. is blown with air in the presence of coils of copper and iron wire which serve as catalysts. At periodic intervals portions of the oil are withdrawn and examined for neutralization number, sediment formation (after 5:1 naphtha dilution) and interfacial tension. The time required for the formation of visible sludge, for the neutralization number to increase to 0.2 mg. per gram, and for the interfacial tension to decrease below 15 dynes per centimeter is reported. A satisfactory oil must have a life of at least 48 hours before reaching any of these three conditions.

This invention is based upon the very interesting finding that a transformer oil made from a mixture of an acid or oleum-treated naphthenic distillate and a hydrofined naphthenic distillate displays superior uninhibited oxidation resistance. Such a blend of oil has an oxidation life materially better than that of either component. This good oxidation resistance is maintained when the conventional 0.3 wt. percent of an oxidation inhibitor such as 2,6-di-tertiary butyl 4-methylphenol is added. With this amount of oxidation inhibitor in the transformer oil blend of this invention, the transformer oil has a Doble oxidation life exceeding 1000 hours and satisfactorily passes the customarily accepted industrial inspections.

Both the acid treated and the hydrofined distillates used in the transformer oil blend of this invention must be derived from naphthenic crudes. Suitable Texas low-cold test (naphthenic) crudes are Webster, Thompson, Sugarland, and Amelia, and can be characterized by the following inspections: Gravity °API 25/29, sulfur 0.2/0.3, vis. SSU at 100° F. 50/80. The distillates can be obtained by conventional atmospheric distillation. Both distillates should have a boiling point in the range of 450° to 900° F. and preferably in the range of 460° to 775° F., an API gravity in the range of 25° to 30°, and

2

preferably in the range of 27° to 28°, a viscosity at 100° F. in the range of 55 to 75 SSU.

The hydrofined component is prepared in a conventional manner by contacting the naphthenic distillate with a hydrofining catalyst in the presence of hydrogen. The temperature of operation is important. Too high a temperature seems to remove too many of the "natural inhibitors," and too low a temperature does not sufficiently correct the instability of the oil. Most advantageously, the temperature used is in the range of 550 to 650° F. During hydrofining, the feed rate is important. Best results are obtained when the feed rate is in the range of 1 to 3 volumes of feed per volume of catalyst per hour (v./v./hour). 500 to 900 standard cubic feet (s.c.f.) per barrel of free hydrogen are used in the hydrofining zone during treatment of the oil. Pressure is not critical and can be of the order of 500 to 750 p.s.i.g. Any suitable hydrofining catalyst can be used such as cobalt molybdate on alumina, and the like. It is preferred to use a 0601P/0301P type catalyst known commercially as Harshaw 0301P and Harshaw 0601P sold by the Harshaw Chemical Company. This hydrofining operation is well known and involves passing the oil at the indicated feed rate and temperature over a fixed bed of the catalyst, while diluted with the indicated amount of hydrogen.

The acid-treated distillate is prepared by the well established sulfuric acid treating process and usually a batch or semi-continuous operation is carried out with one or two "dumps." The acid sludge resulting from the treatment is settled and withdrawn after each dump and prior to the addition of a subsequent dump of acid. Preferred acid-treated distillates are prepared according to this invention when 0.5 to 1.0 lb. per gallon of sulfuric acid in a concentration in the range of 96 to 105% is used at a temperature in the range of 85° to 105° F. and the oil is recovered in yields in the range of 97 to 98 volume percent. The acid-treated distillate should have a —1 to +18 Saybolt color.

It is known to those skilled in the art that the acid treatment of an oil is usually followed by neutralization, as with sodium bicarbonate, followed by steaming at a temperature of 225° to 250° F. and clay contacting or percolation. Both the hydrofined distillate and the acid treated distillate must be treated or contacted with clay in order to arrive at an acceptable product. Clay contacting or percolating is a well established petroleum oil process and involves decolorizing of the oils by contact with finely divided clays such as fuller's earth or bleaching clays. The clays remove soaps from petroleum fractions and increase the oxidation stability. Suitable industrial clays useful in this invention are Bennett-Clark natural clay and Attapulgus. For reasons not quite clear yet, it appears that clay percolation gives better results than clay contacting. Preferably, 0.6 to 1 pound/gal. of absorbent clay is contacted with the distillate oil at a temperature in the range of 250° to 300° F. Clay percolation is carried out at temperatures in the range of 80° to 105° F.

The hydrofined and clay-treated distillate preferably has a boiling point in the range of 460° to 775° F., and API gravity in the range of 27° to 30°, and a viscosity at 100° F. in the range of 55 to 60. The acid and clay-treated distillate preferably has a boiling point in the range of 460° to 775° F., an API gravity in the range of 27° to 30°, and a viscosity at 100° F. in the range of 55 to 60 SSU.

The two distillate oils are blended according to this invention in proportions of 50 to 80 vol. percent of the hydrofined distillate, and 50 to 20 vol. percent of the acid-treated oil. The use of a greater amount of the acid-treated oil is undesirable because it would lead to some loss in oxidation stability and it would be more

expensive. The use of a lesser amount of the acid-treated oil results in a product that is not sufficiently stable when tested in the Doble oxidation test. (Reference: Frank C. Doble, AIEE Transactions, 71, 532 (1952).)

A transformer oil in accordance with the present invention is illustrated by the following examples.

### EXAMPLES

The acid-treated oil used to form the following blends was obtained by treating a 460° to 775° F. distillate obtained from a coastal crude with 2½ vol. percent oleum at 190° F. and recovering the treated oil after one dump in a yield of 97.6%. This acid-treated oil was then neutralized with a 15% sodium bicarbonate solution, followed by two isopropyl alcohol and water washes. The neutralized oil was then steamed at 225° F. using about 0.5 lb. of steam per lb. of oil. The steamed oil was then percolated through 0.6 lb. per gallon of an Attapulgus type clay at 80°–105° F. to arrive at the final product. The final acid-treated oil had a boiling point in the range of 460° to 775° F., an API gravity of 28.1° and a viscosity at 100° F. of 58 SSU.

The hydrofining distillate oil used in these blends was obtained by hydrofining a distillate boiling in the range of 460° to 775° F. obtained from a coastal crude. The hydrofining was carried out over a cobalt molybdate type catalyst sold commercially as Harshaw 0301P or 0601P by the Harshaw Chemical Company. The temperature of hydrofining was 625° F. and the pressure was 750 p.s.i. The feed rate was 1.1 v./v./hr. and the hydrogen rate was 900 s.c.f./bbl. The distillate oil so hydrofined was then treated with a natural type clay sold by the Bennett-Clark Company. 0.8 lb. of clay per gallon of oil was used. The oil was percolated through the clay at a temperature of 300° F. The finished oil had a boiling point in the range of 460° to 775° F., an API gravity of 28.5°, and a viscosity at 100° F. of 56.8 SSU.

These two oils were blended in the proportions indicated in the following tables.

Table I

[Blends (wt. percent)]

|                                                          | 0     | 50    | 70    | 80  | 100   |
|----------------------------------------------------------|-------|-------|-------|-----|-------|
| Hydrofined                                               | 0     | 50    | 70    | 80  | 100   |
| Acid Treated <sup>1</sup>                                | 100   | 50    | 30    | 20  | 0     |
| Doble Oxidation Test:                                    |       |       |       |     |       |
| Uninhibited—Hours:                                       |       |       |       |     |       |
| To 0.2 Neut. No.                                         | 140   | 192+  | 240   | 200 | 40    |
| To 15IFT                                                 | 140   | 192+  | 200   | 150 | 40    |
| To Sludge                                                | 72    | 72    | 72    | 72  | 40    |
| Inhibited (0.31, 2,6 di-tertiary Butyl 4-Methyl Phenol): |       |       |       |     |       |
| Doble Life, Hours                                        | 1,280 | 1,780 | 1,200 | —   | 1,500 |

<sup>1</sup> Oleum treated.

Table II

[Blends (wt. percent)]

|                                                          | 0     | 70  | 50    | 100   |
|----------------------------------------------------------|-------|-----|-------|-------|
| Hydrofined                                               | 0     | 70  | 50    | 100   |
| Acid Treated <sup>1</sup>                                | 100   | 30  | 50    | 0     |
| Doble Oxidation Test:                                    |       |     |       |       |
| Uninhibited—Hours:                                       |       |     |       |       |
| To 0.2 Neut. No.                                         | 140   | 200 | 200   | 40    |
| To 15IFT                                                 | 140   | 200 | 200   | 40    |
| To Sludge                                                | 48    | 48  | 48    | 40    |
| Inhibited (0.31, 2,6 di-tertiary Butyl 4-Methyl Phenol): |       |     |       |       |
| Doble Life, Hours                                        | 1,100 | —   | 1,280 | 1,500 |

<sup>1</sup> 98% Sulfuric acid treated.

It is evident from the above results that exceptionally good oxidation stability is obtained by blending the two oils. This is indeed unexpected as one would expect the oxidation resistance to be intermediate of that of each of the components. The reason for this phenomenon is not yet clear.

It will be appreciated by those skilled in the art that an uninhibited Doble oxidation test life of over 48 hours,

as demonstrated by the above blends, results in a product that is extremely marketable and will find good acceptance in the industry. The inhibitor oxidation test life of the 50–50 blend using 0.3 wt. percent of 2,6 di-tertiary butyl 4-methyl-phenol was 1200 to 1780 hrs., which is considered to be very acceptable performance.

The effect of hydrofining temperature and feed-rate are illustrated by Tables III and IV.

Table III

### EFFECT OF HYDROFINING TEMPERATURE ON DOBLE OXIDATION STABILITY

Catalyst: Cobalt molybdate on alumina  
750 p.s.i.g., 2.0 v./v./hr.  
450 s.c.f./bbl. H<sub>2</sub>  
1.0 lb./gal. Bennett-Clark clay @ 300° F.

| Temp., ° F.           | 475  | 575  | 625 | 675 |
|-----------------------|------|------|-----|-----|
| Sample No.            | 1    | 2    | 3   | 4   |
| Hrs. to 0.2 Neut. No. | 240  | 120  | 272 | 48  |
| Hrs. to Sludge        | 48   | 72   | 72  | 48  |
| Hrs. to 15IFT         | 240+ | 120+ | 72  | 48  |

<sup>1</sup> 0.7 lbs./gal. clay.

<sup>2</sup> Neut. No. 0.31 at 72 hours.

<sup>3</sup> Neut. No. 0.81 at 48 hours.

Table IV

### EFFECT OF FEED ON DOBLE OXIDATION STABILITY

750 p.s.i.g.  
1.0 lb./gal. Bennett-Clark clay @ 300° F.

| Hydrofining Temp.            | 575° F. |      |      | 475° F. |      |
|------------------------------|---------|------|------|---------|------|
| Feed, v./v./hr.              | 1.0     | 2.0  | 3.0  | 1.0     | 2.0  |
| H <sub>2</sub> , s.c.f./bbl. | 856     | 450  | 617  | 920     | 467  |
| Sample                       | 1       | 2    | 3    | 4       | 5    |
| Hrs. to 0.2 N.N.             | 72      | 120  | 144+ | 240     | 240  |
| Hrs. to Sludge               | 72      | 72   | 72   | 48      | 48   |
| Hrs. to 15IFT                | 72      | 120+ | 144+ | 240+    | 240+ |

Having described this invention, what is sought to be protected by Letters Patent is succinctly set forth in the following claims.

What is claimed is:

- An improved transformer oil having, when tested in the absence of inhibitors in the Doble oxidation test for electrical insulating oils, an interfacial tension of at least 15 dynes per centimeter, a neutralization number less than 0.2, and less than a trace of sludge after 48 hours, consisting essentially of a blend of 50–80 volume percent of a hydrofined oil boiling in the range of 460° to 775° F., having an API gravity in the range of 27° to 30°, a viscosity at 100° F. in the range of about 55 to 60 SSU and 50–20 volume percent of an acid-treated oil boiling in the range of 460° to 775° F. having an API gravity in the range of 27° to 30°, a viscosity at 100° F. in the range of 55 to 60 SSU; said hydrofined oil being produced by contacting a distillate boiling in the range of 450° to 900° F. from a naphthenic crude with a hydrofining catalyst at a temperature in the range of 550° to 650° F. and a feed rate in the range of 1 to 3 v./v./hr. in the presence of about 500 to 900 s.c.f./bbl. of free hydrogen, followed by treating the oil so hydrofined with in the range of 0.6 to 1 lb./gal. of an absorbent clay at a temperature in the range of 250° to 300° F., and said acid-treated oil being produced by treating at a temperature in the range of 85 to 105° F. a distillate boiling in the range of 450° to 900° F. from a naphthenic crude with 0.5 to 1.0 lb./gal. of sulfuric acid having a concentration in the range of 96–105% and recovering the acid treated oil in yields in the range of 97 to 98 volume percent and further treating it by neutralization, steaming and clay percolation within the range of 0.6 to 1.0 lb./gal. of an absorbent clay at a temperature in the range of 80° to 105° F.
- An improved blended transformer oil consisting essentially of a blend of 50–80 volume percent of a hydrofined oil made at a temperature in the range of 550–650° F. and boiling in the range of 460° to 775° F., and 50–20

10  
15  
20  
25  
30  
35  
40  
45  
50  
55  
60  
65  
70  
75  
80  
85  
90  
95  
100

volume percent of an acid-treated oil made by contact with 0.5 to 1.0 lb./gal. of sulfuric acid having a concentration in the range of 96-105% and boiling in the range of 460° to 775° F. said hydrofined oil being prepared by contacting a distillate from a naphthenic crude with a hydrofining catalyst in the presence of hydrogen followed by treating the distillate oil so hydrofined with from 0.6 to 1.0 lb./gal. of an absorbent clay, and said acid-treated oil being produced by treating a distillate from a naphthenic crude with sulfuric acid recovering the distillate oil so treated with acid, neutralizing said oil so treated with acid, and treating the oil so neutralized with from 0.6 to 1.0 lb./gal. of an absorbent clay.

3. A transformer oil in accordance with claim 1 wherein said hydrofined oil is produced from a distillate boiling in the range of 460° to 775° F.

4. A transformer oil in accordance with claim 1

wherein said acid-treated oil is produced from a distillate boiling in the range of 460° to 775° F.

5. A transformer oil in accordance with claim 1 wherein said hydrofined oil and said acid-treated oil each have an API gravity in the range of 27° to 28°.

6. A transformer oil consisting of a major amount of a blend in accordance with claim 1 and a minor and oxidation inhibiting amount of 2,6-di-tertiary butyl 4-methyl-phenol.

10

## References Cited in the file of this patent

## UNITED STATES PATENTS

|           |                 |                |
|-----------|-----------------|----------------|
| 1,856,700 | Ford            | May 3, 1932    |
| 2,472,217 | Langan          | June 7, 1949   |
| 2,734,019 | Miller          | Feb. 7, 1956   |
| 2,763,358 | Linn et al.     | Sept. 18, 1956 |
| 2,865,849 | Van Loon et al. | Dec. 23, 1958  |